

# United States Patent [19]

Hill et al.

[11] Patent Number: 5,020,198

[45] Date of Patent: Jun. 4, 1991

- [54] CRIMPED TEXTILE FIBERS AND STUFFER  
BOX APPARATUS AND METHODS FOR  
CRIMPING TEXTILE FIBERS

[75] Inventors: Michael Hill, Ascot, England;  
Walter A. Nichols, Richmond, Va.

[73] Assignee: Filter Materials Ltd., New York,  
N.Y.

[21] Appl. No.: 231,142

[22] Filed: Aug. 10, 1988

[51] Int. Cl.<sup>5</sup> ..... D02G 1/12

[52] U.S. Cl. ..... 28/250

[58] Field of Search ..... 28/250, 251, 265, 263,  
28/264, 268, 269

[56] References Cited

## U.S. PATENT DOCUMENTS

- |           |         |                       |           |
|-----------|---------|-----------------------|-----------|
| 3,226,795 | 1/1966  | Swerdloff et al. .... | 28/265 X  |
| 3,494,522 | 2/1970  | Kim et al. ....       | 225/97    |
| 3,495,752 | 2/1970  | Kim et al. ....       | 225/3     |
| 3,496,260 | 2/1970  | Guenther et al. ....  | 264/156   |
| 3,500,517 | 3/1970  | Dekker et al. ....    | 28/1.5    |
| 3,500,627 | 3/1970  | Kim ....              | 57/140    |
| 3,526,349 | 9/1970  | Moro ....             | 225/97    |
| 3,565,308 | 2/1971  | Slack ....            | 225/97    |
| 3,566,735 | 3/1971  | Greene ....           | 83/344    |
| 3,571,870 | 3/1971  | Dixon ....            | 28/265    |
| 3,577,724 | 5/1971  | Greene ....           | 57/157    |
| 3,595,454 | 7/1971  | Kalwaites ....        | 225/3     |
| 3,726,079 | 4/1973  | Field et al. ....     | 57/155    |
| 3,739,053 | 6/1973  | Yazawa ....           | 264/154   |
| 3,756,484 | 9/1973  | Guenther ....         | 225/97    |
| 3,787,261 | 1/1974  | Heger et al. ....     | 156/84    |
| 3,801,252 | 4/1974  | Waterhouse ....       | 425/304   |
| 3,835,513 | 9/1974  | Stanley ....          | 28/72.14  |
| 3,880,173 | 4/1975  | Hill ....             | 131/269   |
| 3,883,936 | 5/1975  | Stanley ....          | 28/72.14  |
| 3,927,957 | 12/1975 | Chill et al. ....     | 425/131.1 |
| 3,955,255 | 8/1976  | Shields, Jr. ....     | 28/1.6    |

- |           |         |                      |           |
|-----------|---------|----------------------|-----------|
| 3,985,600 | 10/1976 | Blais .....          | 156/229   |
| 3,985,933 | 10/1976 | Mehta et al. .....   | 428/357   |
| 4,129,632 | 12/1978 | Olson et al. .....   | 264/40.1  |
| 4,134,951 | 1/1979  | Dow et al. .....     | 264/147   |
| 4,316,730 | 2/1982  | Eitl .....           | 131/203 X |
| 4,707,896 | 11/1987 | Sowell .....         | 28/250    |
| 4,854,021 | 8/1989  | Reinehr et al. ..... | 28/263    |

## FOREIGN PATENT DOCUMENTS

- |         |         |                  |        |
|---------|---------|------------------|--------|
| 7324417 | 7/1970  | Japan .....      | 28/264 |
| 1207733 | 10/1970 | United Kingdom . |        |
| 1260957 | 1/1972  | United Kingdom . |        |
| 1301242 | 12/1972 | United Kingdom . |        |
| 1339496 | 12/1973 | United Kingdom . |        |
| 1442593 | 7/1976  | United Kingdom . |        |

#### OTHER PUBLICATIONS

Filter Materials Ltd. brochure, 1986.

*Primary Examiner*—Werner H. Schroeder

*Assistant Examiner—John J. Calvert*

## ABSTRACT

An improved stuffer box used for crimping textile fibers, particularly fibrillated polyolefin films. The width of the stuffer box is related to the linear density of the fiber bundles to be crimped whereby there is one millimeter of width for each fiber binder size in the range of from about 200 to about 750 denier. Pressure controlled hinged lid or fixed lid exit orifices may be employed. Also employed may be a distributing device for applying additive material to the textile fibers prior to crimping to enhance the crimping operation or to enhance the end use of the crimped fiber or both. Fibrillated polyolefin materials that are crimped in accordance with the invention are adapted for use as filter materials in smoking articles.

**45 Claims, 5 Drawing Sheets**



FIG. 1





FIG. 2

FIG. 3



FIG. 4



FIG. 5



**CRIMPED TEXTILE FIBERS AND STUFFER BOX APPARATUS AND METHODS FOR CRIMPING TEXTILE FIBERS**

**BACKGROUND OF THE INVENTION**

This invention relates to a method and apparatus for crimping textile fibers, and particularly to crimping fibrillated polyolefin materials for use as filter materials for tobacco-containing smoking articles.

Texturizing textile fibers, i.e., imparting a crimp into the fibers, using the "stuffer box" principle is well known. Crimping occurs by advancing the fiber at a given rate of speed into an enclosed box whereupon the fiber rapidly decelerates; hence the term stuffing. The stuffer box typically has either a lid that is hinged by one of a variety of techniques, or is fixed with a preset exit orifice, whereby when the box is filled with fiber and a certain predetermined pressure is achieved within the box, fibers will exude out; for example, when the pressure overcomes the forces holding the hinged lid closed, or, if the lid is fixed, when the pressure forces the fiber out the exit orifice.

The effect of the varying pressures inside the box is to impart crimps into the textile fibers. A primary crimp occurs when the individual fibers obtain a wavy shape, for example, during rapid deceleration when the fibers hit the end wall of the stuffer box or the preceding crimped fiber. A secondary crimp occurs when the collapsed individual fibers begin to fold in on themselves inside the stuffer box.

Control of the pressure within the stuffer box is critical because it determines the regularity and nature of the primary crimp, i.e., the crimp frequency and amplitude. Generally, the frequency and amplitude are related so that as the frequency increases, the amplitude decreases. Control of the pressure is generally achieved by careful control of the movement of the hinged lid of the box, or by designing the fixed exit geometry of the box to known preset values such that the pressure drop across the box is known and gives the required fiber crimp characteristics.

Although the pressure exerted on the fibers by the hinged lid may be achieved by a variety of techniques, most commercially available systems employ a means of mechanically exerting pressure on the lid to preset values using pneumatic or hydraulic cylinders or actuators, or a known mass (weight) or masses.

Other factors that may affect the nature of the crimp achieved in the textured fiber include the overall geometry and volume of the box and surface frictional characteristics of the internal surfaces of the box, the diameter and surface characteristics of the feed rollers advancing and forcing the fibers into the box and the pressure with which these feed rollers are held together, the temperature of the box, the characteristics of the fibers being crimped and any pretreatment of the fibers. The characteristics of the fibers may vary with, for example, the chemical composition, fiber size and shape, fiber size distribution, number of fibers, and temperature. Pretreatment techniques may include, for example, thermal treatment or adding lubricants, anti-static finishes, oils, moisture, etc.

Conventional stuffer boxes embody a principle relating the width of the stuffer box to the total number of textile fibers or bundles in the tow to achieve desired crimp levels. Generally, for every millimeter of box width the fiber bundle to be crimped should have a size

in the range of from about 1000 to about 1800 denier (hereinafter referred to as the "conventional rule"). Accordingly, for a fiber network having a total linear density of 40,000 denier, the stuffer box should have a width in the range of from about 22.2 mm to about 40.0 mm. Conventional equipment not complying with the conventional rule has been found to provide tows having unacceptable crimp characteristics.

It also is known to use fibrillated polyolefin films and 10 form them into filter materials by forming them into a bloomed flocculated mass which is then formed into a filter rod by using conventional filter rod making equipment. These fibrillated polyolefin materials have an interconnected network of fibers and strands, including 15 fibers connected to the network only at one point. These materials have been subjected to the conventional crimping process with some success.

However, one of the problems with the conventional stuffer boxes for crimping fibrillated polyolefin tow is 20 that the crimp amplitude and frequency has not been sufficient to impart adequate filtration capabilities into such materials when formed into filter rods in a conventional manner.

Notwithstanding years of development efforts, there 25 is no commercial use of a filter for smoking articles comprising a fibrillated polyolefin material that provides the advantages and benefits associated with conventional cellulose acetate filter materials used in smoking articles, and particularly, tobacco-containing cigarettes.

Accordingly, there is a continuing need for apparatus and methods for processing fibrillated polyolefin materials to produce filter materials appropriate for use in smoking articles that is more effective, and easier and cheaper to manufacture and form into filters than conventional cellulose acetate materials.

**SUMMARY OF THE INVENTION**

It is an object of this invention to provide an improved stuffer box for imparting crimps into a tow of textile fibers to provide an increased number of crimps per inch in the tow material. It is another object to provide a crimped textile material, including but not limited to fibrillated polyolefin films, having an increased number of crimps per inch.

It is another object of this invention to provide an improved stuffer box for imparting crimps into a tow of fibrillated polyolefin materials that can be adapted for forming into filter rods for use in smoking articles. It is another object to provide additives prior to crimping such materials to improve the smoking and taste characteristics of such filter rods.

It is another object of this invention to provide improved processing of fibrillated polyolefin film tow for forming crimps in the tow.

In accordance with the present invention, there is provided a stuffer box having a configuration that differs significantly from the conventional rule and provides crimped fiber bundles that have the acceptable crimp characteristics suitable for use in the manufacture of textured fibers for conventional purposes. Broadly, the invention comprises a stuffer box having an entry width whereby there is one millimeter of width for each fiber bundle size of about 200 to about 750 denier, more preferably about 500 denier.

The stuffer box is preferably configured with a hinged lid wherein the hinge is a self-exhausting pneu-

matic cylinder adapted for urging the lid closed. Conventional feed rollers for advancing the fibers and exerting pressure on the fibers may be used to feed the textile fibers into the stuffer box. Means for cooling the feed rollers with, e.g., water, compressed air, may be provided.

The stuffer box of the present invention is particularly applicable for processing textile fiber filaments interconnected in a network configuration or fiber filaments interconnected in the main on a network configuration but having some fibers connected into the network by one connection point only, or an interconnected network of fiber having discrete fibers of the same kind or different (i.e., chemically different, different in size or geometry) enmeshed in the main fiber network, or an interconnected network of fibers having discrete inclusion of additives separate to or coating the fibers comprising the network, or any combination of the above. More particularly, the stuffer box of the present invention is adapted for texturizing fibrillated polyolefin fibers of the type described in U.S. Pat. No. 3,880,173, its corresponding U.K. Patent 1,442,593, or copending and, commonly assigned U.S. application Ser. No. 07/231,144, (PM-1301), the disclosures of which are hereby incorporated by reference.

In accordance with another aspect of the invention, there is provided a method for processing the foregoing fibers by adding one of a variety of chemical additives applied prior to subjecting the fibers to the stuffer box of the present invention to enhance the resultant range of final texturized properties of the fibers. Such additives also may be used to influence smoke and taste characteristics when the texturized fiber tow is used in filter tow applications, particularly for tobacco-containing cigarettes. Such additives may be selected from among the group consisting of oils, fatty acid esters, waxes, esters of alcohols, ionic and non ionic surfactants, or blends of the same.

The present invention permits the crimping of interconnected fibrous networks of fiber to levels desirable to facilitate the manufacture of cigarette filter tow and further confers the ability to influence subjective responses on cigarettes fitted with filter rods made from the treated crimped fiber tow. The present invention further provides for imparting a higher crimp frequency than is obtainable from conventional apparatus.

The improved nature of the resultant crimped fiber tow is observed from the crimp frequency and amplitude, wherein the crimp frequency is defined as the number of complete adjacent peaks and troughs per unit length, in units of cycles per inch, and the crimp amplitude is defined as the total vertical distance between adjacent peaks and troughs in the crimped fiber.

The improvement is further observed from the improved Tow Yields for fibrillated polyolefin materials made by the present invention that are formed into filter lengths using conventional filter rod making equipment such as that used for forming cellulose acetate tow into filter materials. Tow Yields are obtained from the following expression:

$$\text{Tow Yield} = \frac{\text{Pressure drop (mm WG)}}{\text{Net Weight of Fiber in rod (mg)}} \times 100\%.$$

The Net Weight is measured in units of milligrams for a given length of filter rod. The pressure drop is measured in millimeters of Water Gauge at an air-flow of 1,050 ml per minute through the net weight of rod. Higher Tow Yields correspond to more randomly dis-

persed free ends and an improved fibrous strand network and, hence, a more efficient use of the polyolefin materials.

#### BRIEF DESCRIPTION OF THE DRAWINGS

The above and other objects and advantages of the invention will be apparent upon consideration of the following detailed description, taken in consideration with the accompanying drawings, in which like reference characters refer to like parts throughout, and in which:

FIG. 1 is an elevated perspective view of a stuffer box in accordance with an embodiment of the present invention;

FIG. 2 is a side view taken along line 2—2 of FIG. 1;

FIG. 3 is a top view of FIG. 1;

FIG. 4 is an illustrative schematic view of a fibrillation apparatus incorporating the stuffer box of the present invention; and

FIG. 5 is a schematic cross sectional side view of a stuffer box in accordance with an embodiment of the present invention.

#### DETAILED DESCRIPTION OF THE INVENTION

As shown in FIGS. 1-3, and 5, illustrative embodiments of this invention include stuffer box 10 adapted for imparting crimps to textile material 20 thereby forming crimped textile material 22. Associated with stuffer box 20 are feed rollers 30 which advance material 20 into opening 8 of stuffer box 10. Feed rollers 30 may be urged together with a loading sufficient to maintain frictional contact with material 20 and thereby advance material 20 into opening 8 of box 10. For example, pneumatic cylinders may be used to exert a force of from about 0.1 to about 5 bars to urge the rollers together. Feed rollers are preferably of about the same dimensions and are about the same width as opening 8 of box 10, although there may be some differences, for example, upper roller 30 being about the same width as opening 8 and lower roller 30 being somewhat wider than opening 8.

Feed rollers 30 also may have an associated cooling mechanism which may be a source of compressed air 34 and vents 32 directed to one or both of feeding rollers 30 (only one vent shown in the Figs.). Other sources of cooling feed rollers 30 that will not adversely affect textile material 20 for its intended uses may be used, e.g., water, oil, refrigerated air and the like.

Stuffer box 10 further includes lid 12 which is connected to box 10 at hinge 14, base 13 and self-exhausting pneumatic cylinder 40 which is capable of exerting a selectable level of force so that when that level of force is overcome, the cylinder will collapse and translate. Thus, hinged lid 12 is maintained urged closed by cylinder 40 which is adjusted to exert on lid 12 the preselected level of force for the particular crimping operation on the given textile fiber. For example, and with reference to Examples 3-9, predetermined threshold forces in a range of from about 1.0 kgf to about 50 kgf may be used.

Optionally, source of additive 50 and distribution means 52 may be provided at an appropriate location, e.g., prior to or subsequent to feed rollers 30 (only the former is shown in the Figs.). Distribution means 52 includes a metering means for controlling the rate of application of the additive to the textile material 20.

Stuffer box 10 has entry width  $w$ , entry height  $h$ , and length 1, that are selected for the given linear density of the textile material as are described above and below in connection with the Examples. The exit width is typically about the same as the entry width and the exit height for a hinged lid stuffer box is dependent upon the desired pressures to be generated inside the stuffer box and the force selected for cylinder 40. Such heights are generally a fraction of the entry height, e.g., 63%.

Referring to FIG. 4, uns fibrillated polyolefin film 100 is passed through orientation oven 110 and then over pinned roller 120 having a plurality of rows 114 of pins (not shown) spaced about the circumference of roller 120, thereby providing fibrillated film 102. Fibrillated film 102 is then passed under additive distribution means 52 and between feed rollers 30 and into stuffer box 10 for the crimping operation in accordance with the present invention.

Referring to FIG. 5, stuffer box 10 comprises base 13, opening 8, lid 12, and hinge 14. Hinge 14 is integral with upper roller 30 and is shown in its upper and unloaded condition. Cylinder 40 has extension arm 42 which is in an unloaded condition. When cylinder 40 is actuated, arm 42 will extend downwardly and contact receptacle 44 which will cause lid 12 to rotate about hinge 14 until lid 12 contacts base 13. When material 20 (not shown in FIG. 5) is advanced into box 10 and the pressure risen above the predetermined threshold force exerted by cylinder 40, lid 12 will rotate upwardly and release crimped material 22 (not shown in FIG. 5).

The method and apparatus of the present invention is further described in connection with the following examples.

## EXAMPLES

Each of following examples were prepared from following blend of polyolefin materials:

92% polypropylene homopolymer, melt index 1.8 (230° C., 2.16 kgf)

7% low density polyethylene, melt index 1.0 (190° C., 2.16 kgf)

1% polypropylene (of the same type as above) masterbatch, containing 25% titanium dioxide (rutile grade, fine crystal structure, micronized grade).

These materials were mixed and extruded using a known blown film technique to produce a film of 35  $\mu$  thickness. This film was then slit into six portions of substantially equal width, stacked, and oriented in a longitudinal direction with a stretch ratio of 8:1 to produce films of 12.4  $\mu$  thickness. The oriented films were then passed around part of the periphery of a pinned fibrillating roller passed into a stuffer box in accordance with the present invention for the texturizing operation for crimping the fibrillated film.

In each example, the pinned roller used had a diameter of 190 mm at the roller surface, and the angle of rake of the pins was 60 degrees (relative to the tangent). There were 180 lines of pins in paired rows to form 90 double rows of pins in a space-staggered relationship and the pin diameter was 0.4826 mm. The pins had a pin projection length of about 1.0 mm, the pin projection length being measured from the pin tip to the roll surface in a plane passing through the roll axis. The double rows extended across the roller having a chevron pattern.

The configuration of the stuffer box and the processing parameters for the texturizing operation, and the resulting crimp parameters are set forth in Table I.

TABLE I

| Parameter                                     | PROCESSING PARAMETERS |                 |                 |                     |                                                                                  |                                           |                                         |                                            |                                         |
|-----------------------------------------------|-----------------------|-----------------|-----------------|---------------------|----------------------------------------------------------------------------------|-------------------------------------------|-----------------------------------------|--------------------------------------------|-----------------------------------------|
|                                               | Examples              |                 |                 |                     |                                                                                  |                                           |                                         |                                            |                                         |
|                                               | Ex. 1                 | Ex. 2           | Ex. 3           | Ex. 4               | Ex. 5                                                                            | Ex. 6                                     | Ex. 7                                   | Ex. 8                                      | Ex. 9                                   |
| Total Tow Denier                              | 38,000                | 60,000          | 36,000          | 40,000              | 40,000                                                                           | 40,000                                    | 41,000                                  | 38,000                                     | 36,500                                  |
| Input Speed of Tow (m/min)                    | 138                   | 60              | 138             | 138                 | 138                                                                              | 138                                       | 138                                     | 138                                        | 138                                     |
| Stuffer Box Width (mm)                        | 80                    | 40              | 80              | 80                  | 80                                                                               | 80                                        | 80                                      | 80                                         | 101.6                                   |
| Stuffer Box Entry Height (mm)                 | 20                    | 12              | 4               | 4                   | 4                                                                                | 4                                         | 4                                       | 8                                          | 20                                      |
| Stuffer Box Length (mm)                       | 175                   | 160             | 165             | 165                 | 165                                                                              | 165                                       | 165                                     | 175                                        | 130                                     |
| Pressure on Hinged Lid of Stuffer Box (kgf)   | 10                    | 0.8 bar         | 10              | 15                  | 12.5                                                                             | 12                                        | 15                                      | 0.5 BAR applied to top and bottom surfaces | 10                                      |
| Pressure on Feed Rollers of Stuffer Box (bar) | 2                     | 2.5             | 3               | 3                   | 3                                                                                | 3                                         | 3                                       | 3                                          | 3                                       |
| Feed Roller Diameter (mm)                     | 80                    | 200             | 80              | 80                  | 80                                                                               | 80                                        | 80                                      | 150                                        | 80                                      |
| Box Temperature (°C.)                         | 40                    | 20              | 60              | 60                  | 60                                                                               | 60                                        | 60                                      | Ambient                                    | 40                                      |
| Box Material                                  | Brass                 | Stainless Steel | Stainless Steel | Stainless Steel     | Stainless Steel                                                                  | Stainless Steel                           | Stainless Steel                         | Stainless Steel                            | Brass                                   |
| Feeder Roller Cooling                         | None                  | Water           | Air             | Air                 | Air                                                                              | Air                                       | Air                                     | Water                                      | None                                    |
| Additives Applied to Tow Prior To Crimping    | None                  | None            | Deionized Water | Poly-glycol Ester** | Glyceral Tri-acetate (C <sub>9</sub> H <sub>14</sub> O <sub>6</sub> ), 30 ml/min | Blend of fatty acid ester and mineral oil | PoE Sorbitan Mono-stearate*** 20 ml/min | Poly-glycol Ester** 40 ml/min              | Deionised water; 20 ml/min Cirrasol**** |

TABLE I-continued

| Parameter                      | PROCESSING PARAMETERS |       |       |       |       |           |       |       |       |
|--------------------------------|-----------------------|-------|-------|-------|-------|-----------|-------|-------|-------|
|                                | Examples              |       |       |       |       |           |       |       |       |
|                                | Ex. 1                 | Ex. 2 | Ex. 3 | Ex. 4 | Ex. 5 | Ex. 6     | Ex. 7 | Ex. 8 | Ex. 9 |
| Mean Crimp Frequency (cpi)     | 14.9                  | *     | 58.4  | 54.5  | 52.8  | 20 ml/min | 43.2  | 57.7  | 21.4  |
| Mean Crimp Amplitude ( $\mu$ ) | 592                   | *     | 360   | 382   | 380   | 58.2      | 344   | 428   | 512   |

\*Could not be determined without destroying the nature of the crimp; tow exiting the box contained welded bands of fiber that could not be separated for making measurements.

\*\*Brand name LW1177, available from Henkel-Nopco, Ltd., Nopco House, Kirkstall Road, Leeds, England.

\*\*\*Brand name Tween 21, available from ICI Speciality Chemicals, Cleeve Road, Leatherhead, Surry, England.

\*\*\*\*Brand name DS5676, available from ICI Speciality Chemicals, Cleeve Road, Leatherhead, Surry, England.

The fibrillated material was then formed into a filter rod using conventional filter rod forming apparatus for example, model KDF-2 manufactured by Hauni Werke Korber & Co., Hamburg, Germany, wherein the tow is formed into a bloomed flocculent mass having the identified crimp characteristics, and processed by the filter making apparatus into a rod having a circumference of 24.55 mm and a length of 66 mm. Other filter dimension could be obtained.

The results of the evaluation of the filter material constructed from the fibrillated material of the examples are set forth in Table II. The low yield and high yield values respectively correspond to the minimum point and the maximum point on the capability curve, which curve compares relative pressure drop for changes in the net weight of tow material in a uniformly dimensioned filter rod. All of Examples 3-9 provided a tow yield that reflected a significant improvement over the crimped fibrillated polyolefin filter rods obtained by prior known devices as in Examples 1 and 2 and over conventional cellulose acetate filters.

15 forth in Table I, and produced rows characterized by a high crimp frequency, a low crimp amplitude and high tow yields suitable for use as filter materials in smoking.

One skilled in the art will appreciate that the present invention can be practiced by other than the described embodiments, which are presented for purposes of illustration and not of limitation, and the present invention is limited only by the claims which follow.

We claim:

1. Apparatus for texturizing advancing textile fibers having fiber bundles comprising a stuffer box having: an entry aperture having a height of from about 2 to about 20 mm and a width of one millimeter for each fiber bundle having a linear density in the range of from about 200 to about 750 denier; means for accumulating advancing textile fibers inside the stuffer box thereby to crimp the textile fibers; an exit orifice; and means for releasing accumulated crimped textile fibers through the exit orifice when the pressure of

TABLE II

|                           | TOW YIELDS |         |       |       |       |       |       |        |       |
|---------------------------|------------|---------|-------|-------|-------|-------|-------|--------|-------|
|                           | Ex. 1*     | Ex. 2** | Ex. 3 | Ex. 4 | Ex. 5 | Ex. 6 | Ex. 7 | Ex. 8* | Ex. 9 |
| <u>LOW YIELD</u>          |            |         |       |       |       |       |       |        |       |
| Mean Pressure Drop (mmWG) | 141        |         | 219   | 252   | 300.5 | 267   | 265.5 | 221    | 188   |
| Net Weight of Rod (mg)    | 323        |         | 300   | 327   | 261.5 | 305   | 343   | 313    | 286   |
| Yield (%)                 | 44         |         | 73    | 77    | 83    | 68    | 77    | 71     | 66    |
| <u>HIGH YIELD</u>         |            |         |       |       |       |       |       |        |       |
| Mean Pressure Drop (mmWG) |            | 268     | 339   | 376   | 264   | 353.5 |       | 262    |       |
| Net Weight of Rod (mg)    |            | 333     | 371   | 396.2 | 341   | 386   |       | 334    |       |
| Yield (%)                 |            | 80      | 91    | 95    | 77    | 91    |       | 78     |       |

\*Data represents an overall view of the low and high yield points on the capability curve.

\*\*No data obtained.

The crimper box of Example 1 was wider than the width dictated by the conventional rule, had a high box entry height and a standard roller diameter, had no additives or roller cooling, and produced a tow characterized by low yields, low crimp frequency and high crimp amplitude, and shows the effect of and indicates the benefit of the application of additives to the fiber prior to crimping. The crimper box of Example 2 was constructed to a width dictated by the conventional rule, had a medium box entry height, a large roller diameter and roller cooling, but did not have additives, and produced a tow having fused sections which is useless for smoke filtering applications.

The crimper boxes of Examples 3-9 constructed in accordance with various embodiments of the present invention, had wider widths than the width dictated by the conventional rule and the other parameters as set

55 the accumulated fibers exceeds a predetermined threshold force.

2. The apparatus of claim 1, further comprising means for distributing an additive material on the textile material prior to the opening of said stuffer box.

3. The apparatus of claim 2, wherein said additive material is selected from among the group consisting of oils, fatty acid esters, waxes, esters of alcohols, ionic and non ionic surfactants, or a mixture thereof.

4. The apparatus of claim 1, wherein said first predetermined force is in a range of from about 1.0 to about 50 kgf.

5. The apparatus of claim 1 further comprising means for advancing textile fibers into the entry aperture, said means comprising a pair of opposing feed rollers being

urged together by a second predetermined force in a range of from about 0.1 to about 5.0 bar.

6. The apparatus of claim 1 wherein the textile fiber further comprises a fibrillated polyolefin film having a linear density of from about 15,000 to about 50,000 denier, and said first width being within a range from about 30 to about 110 mm. 5

7. The apparatus of claim 6 wherein the first predetermined force is in the range of from about 1.0 to about 50 kgf. 10

8. The apparatus of claim 6 wherein said first width further comprises from about 70 to about 110 mm.

9. The apparatus of claim 8 wherein the first predetermined force is in the range of from about 1.0 to about 50 kgf. 15

10. The apparatus of claim 9 wherein the entry aperture further comprises a width of one millimeter for each fiber bundle having a linear density in the range of from about 400 to about 600 denier.

11. The apparatus of claim 1 wherein the accumulating means, exit orifice, and releasing means further comprise: 20

a lid for covering the exit orifice

a hinge connecting the lid to the stuffer box so that the lid covers the exit orifice; 25

means for urging the lid closed against the exit orifice with the first predetermined force, the urging means being responsive to the pressure of the accumulated textile fibers inside the stuffer box so that when the pressure exceeds the predetermined threshold force, the urging means permits the lid to move and crimped textile fibers to pass through the exit orifice. 30

12. The apparatus of claim 11 wherein said first predetermined force is in a range of from about 1.0 about 50 kgf. 35

13. The apparatus of claim 11 further comprising means for maintaining the stuffer box at a temperature of from about 20 to about 90° C.

14. The apparatus of claim 11 further comprising means for advancing textile fibers into the entry aperture, said means comprising a pair of opposing feed rollers being urged together by a second predetermined force in a range of from about 0.1 to about 5.0 bar. 40

15. The apparatus of claim 11 wherein the textile fiber further comprises a fibrillated polyolefin film having a linear density of from about 15,000 to about 50,000 denier, and said first width being within a range from about 30 to about 110 mm. 45

16. The apparatus of claim 15 wherein the first predetermined force is in the range of from about 0.1 to about 50 kgf. 50

17. The apparatus of claim 16 wherein said first width further comprises from about 70 to about 110 mm.

18. Apparatus for texturizing advancing textile fibers having fiber bundles comprising a stuffer box having an entry aperture including a first width and a first height, and an exit orifice, said first width being within a range based upon the linear density of the advancing textile fibers whereby there is one millimeter of width for each fiber bundle having a linear density in the range of from about 400 to about 600 denier, said first height being from about 2 to about 20 mm, said exit orifice having a retention condition and a release condition, said retention condition being adapted to accumulate within the stuffer box the advancing textile fiber thereby to crimp said fiber, aid release condition being adapted to release through said exit orifice the crimped textile fiber when 65

the pressure of the advancing accumulating textile fiber exceeds a first predetermined threshold force, the exit orifice further comprising

a lid for closing the exit orifice so that crimped textile fiber will accumulate within the stuffer box and for opening so that crimped textile fiber may be released through the exit orifice; a hinge connecting the lid to the stuffer box; and a pneumatic cylinder exerting a force on the lid, thereby urging the lid closed, whereby when the pressure within the stuffer box exceeds the predetermined force, the pneumatic cylinder will permit the lid to rotate about the hinge to open so that crimped textile fiber will pass through the exit orifice until the pressure inside the stuffer box falls below the predetermined pressure.

19. A method of crimping fibrillated polyolefin materials comprising:

providing a tow of fibrillated polyolefin material having bundles;

providing a stuffer box having an entry aperture and an exit orifice, the entry aperture having a height of from about 2 to about 20 mm and a width,

selecting the stuffer box entry aperture width based upon the linear density of the material whereby there is one millimeter of width for each bundle of material having a linear density in the range of from about 200 to about 750 denier;

advancing the tow into the entry aperture of the stuffer box;

accumulating material in the stuffer box thereby crimping the material;

releasing accumulated crimped material through the exit orifice when the pressure of the accumulated material exceeds a predetermined force.

20. The method of claim 19 further comprising distributing an additive material on the polyolefin material prior to the entry aperture, the additive material being selected from among the group consisting of oils, fatty acid esters, waxes, esters of alcohols, ionic and non-ionic surfactants, and mixtures thereof.

21. The method of claim 19 wherein selecting the width further comprises providing one millimeter of width for each bundle of material having a linear density in the range of from about 400 to about 600 denier.

22. The method of claim 19 further comprising releasing the accumulated fibers when the pressure exceeds a force in the range of from about 1.0 to about 50 kgf.

23. The method of claim 19 further comprising maintaining the stuffer box at a temperature of from about 20 to about 90° C.

24. The method of claim 19 wherein advancing the polyolefin material further comprises passing the material between a pair of opposing feed rollers urged together by a force in a range of from about 0.1 to about 5.0 bar.

25. The method of claim 19 wherein the polyolefin material has a linear density in the range of from about 15,000 to about 50,000 denier and wherein the entry aperture width is in the range of from about 30 to about 110 mm.

26. The method of claim 25 wherein the entry aperture width is in the range of from about 70 to about 100 mm.

27. The method of claim 19 wherein providing the two further comprises providing a polyolefin material having a linear density in the range of from about 15,000 to about 50,000 denier, selecting the entry aperture

further comprises providing a width in the range of from about 70 to about 110 mm, and wherein advancing the polyolefin material further comprises passing the material between a pair of opposing feed rollers urged together by a force in a range of from about 0.1 to about 5.0 bar, the method further comprising:

5 distributing an additive material on the polyolefin material prior to the entry aperture, the additive material being selected from among the group consisting of oils, fatty acid esters, waxes, esters of 10 alcohols, ionic and non-ionic surfactants, and mixtures thereof;

releasing the accumulated fibers when the pressure exceeds a force in the range of from about 1.0 to about 50 kgf; and

maintaining the stuffer box at a temperature of from about 20 to about 90° C.

28. A crimped polyolefin material produced by the method of claim 27.

29. The method of claim 19 wherein accumulating material and releasing accumulated material further comprise:

providing the exit orifice with a lid connected to the 25 stuffer box;

biasing the lid closed against the exit orifice; and opening the lid when the pressure of the accumulated material exceeds the predetermined force, thereby releasing accumulated crimped material through the exit orifice.

30. The method of claim 29 further comprising distributing an additive material on the polyolefin material prior to the entry aperture, the additive material being selected from among the group consisting of oils, fatty 35 acid esters, waxes, esters of alcohols, ionic and non-ionic surfactants, and mixtures thereof.

31. The method of claim 29 wherein selecting the width further comprises providing one millimeter of width for each bundle of material having a linear density in the range of from about 400 to about 600 denier.

40 32. The method of claim 29 further comprising biasing the lid closed with the second predetermined force being in the range of from about 1.0 to about 50 kgf.

33. The method of claim 29 further comprising maintaining the stuffer box at a temperature of from about 20 45 to about 90° C.

34. The method of claim 29 wherein advancing the polyolefin material further comprises passing the material between a pair of opposing feed rollers urged together by a force in a range of from about 0.1 to about 5.0 bar.

50 35. The method of claim 29 wherein the polyolefin material has a linear density in the range of from about 15,000 to about 50,000 denier and wherein the entry aperture width is in the range of from about 30 to about 110 mm.

36. The method of claim 35 the entry aperture width is in a range of from about 70 to about 110 mm.

55 37. The method of claim 29 wherein providing the tow further comprises providing a polyolefin material having a linear density in the range of from about 15,000 to about 50,000 denier, selecting the entry aperture width further comprises a width in the range of from about 70 to about 110 mm, and wherein advancing the polyolefin material further comprises passing the material between a pair of opposing feed rollers urged together by a force in a range of from about 0.1 to about 5.0 bar, the method further comprising:

distributing an additive material on the polyolefin material prior to the entry aperture, the additive material being selected from among the group consisting of oils, fatty acid esters, waxes, esters of alcohols, ionic and non-ionic surfactants, and mixtures thereof;

biasing the lid closed with a force in the range of from about 1.0 to about 50 kgf; and

maintaining the stuffer box at a temperature of from about 20 to about 90° C.

38. A crimped polyolefin material produced by the method of claim 37.

39. A system for crimping fibrillated polyolefin materials comprising:

15 a tow of fibrillated polyolefin material having a linear density in the range of from about 15,000 to about 50,000 denier and a plurality of fiber bundles;

a stuffer box having an entry aperture and an exit orifice, the entry aperture having a height in the range of from about 23.0 to about 20 mm and a width of one millimeter for each fiber bundle having a linear density in the range of from about 200 to about 750 denier and a height in the range of from about 2.0 to about 20 mm, a means for accumulating within the stuffer box the advancing material thereby to crimp the material, and a means for releasing accumulated crimped material when the pressure of the accumulated material in the stuffer box exceeds a predetermined threshold force; and

means for advancing the polyolefin material into the entry aperture.

40. The system of claim 39 wherein the stuffer box releasing means further comprises:

a lid for covering the exit orifice; a hinge connecting the lid to said stuffer box to cover the exit orifice; and

means for urging the lid closed against the exit orifice with the first predetermined force, whereby when the pressure within the stuffer box exceeds the first predetermined force, the urging means will permit the lid to move to uncover the exit orifice so that crimped material may pass through the exit orifice until the pressure inside the stuffer box falls below the first predetermined force.

41. The system of claim 39 further comprising means for distributing an additive material on the polyolefin material prior to the entry aperture, the additive material being selected from among the group consisting of oils, fatty acid esters, waxes, esters of alcohols, ionic and non-ionic surfactants, or a mixture thereof.

42. The system of claim 39 wherein the stuffer box entry aperture further comprises one millimeter of width for each bundle having a linear density in the range of from about 400 to about 600 denier.

43. The system of claim 39 wherein the predetermined threshold force is in the range of from about 1.0 to about 50 kgf.

44. The system of claim 39 wherein the advancing means further comprises a pair of opposing feed rollers being urged together by a force in a range of from about 0.1 to about 5.0 bar.

45. The system of claim 39 wherein the stuffer box entry aperture further comprises one millimeter of width for each fiber bundle having a linear density in the range of from about 400 to about 600 denier, the predetermined threshold force is in the range of from about 1.0 to about 50 kgf, and the advancing means

further comprises a pair of opposing feed rollers being urged together by a force in a range of from about 0.1 to about 5.0 bar, the system further comprising means for distributing an additive material on the polyolefin material prior to the entry aperture, the additive material

5

being selected from among the group consisting of oils, fatty acid esters, waxes, esters of alcohols, ionic and non-ionic surfactants, or a mixture thereof.

\* \* \* \* \*

10

15

20

25

30

35

40

45

50

55

60

65